

Oct. 29, 1968

C. E. HOING  
METHOD FOR DRY SORTING THE CONSTITUENTS  
OF A HOMOGENEOUS MIXTURE  
Filed Feb. 20, 1967

3,407,929



INVENTOR

CHRISTINE ELISABETH HOING

By Young & Thompson  
ATTYS.

1

3,407,929

METHOD FOR DRY SORTING THE CONSTITUENTS  
OF A HOMOGENEOUS MIXTURE

Christine Elisabeth Hoing, Rue de Beaupreau 29,  
Sainte-Genevieve, France  
Filed Feb. 20, 1967, Ser. No. 617,301  
Claims priority, application France, Mar. 1, 1966,  
51,428; Aug. 5, 1966, 72,181  
4 Claims. (Cl. 209—3)

## ABSTRACT OF THE DISCLOSURE

The constituents of a homogeneous granular mixture are dry sorted by passing the mixture down a first inclined perforated chute, blowing a gas through the perforations in the chute to fluidize the granular particles and passing the fluidized mixture down a second inclined perforated chute along which the granular particles are sorted and deposited through the perforations according to their specific weights.

According to the present invention there is provided a method for dry sorting the constituents of a homogeneous mixture.

When a homogeneous mixture of heterogeneous granular substances of different specific weights are placed on a sloping surface, the mixture tends to flow down the surface due to the force of gravity and due to the heavier particles being concentrated in the lower layers of the stream and the lighter higher layers toppling over the lower heavier layers.

A similar result is obtained by subjecting a homogeneous mixture to an upwardly directed stream of gas passing through said mixture.

However, in the present state of the art, dry sorting a homogeneous mixture in accordance with the specific weights of the constituent granular particles by using either of the above principles applied alone or in combination has not found any satisfactory practical solution.

A combination of the two principles is sometimes effected when it is required to remove the heavier product located in the lower portion of the stream of the granular products through a succession of ports located in the area subjected to a blast of air. However, the extraction thus performed disturbs considerably the sorting of the products in the actual area in which said extraction is executed, which leads to a reduction in the efficiency of the sorting procedure.

Considering the constituents of an initial mixture of granular particles sorted in accordance with their specific weights, I will term efficiency of the sorting executed in accordance with my invention as the ratio of the weight of the granular particles of a constituent in the mixture and the weight of the granular particles of the constituent which have actually been sorted from the mixture, disregarding the particles which should have been incorporated with other sorted constituents.

An object of my invention is to obtain a high efficiency.

Further objects of my invention consist in providing a sorting method which is also economical in energy expenditure and in providing a sorting method which may be conveniently executed in a static plant. A still further object consists in retaining the product in a dry condition without requiring as in the case of the moist methods, any subsequent drying.

The perfecting of my invention has been obtained by an accurate investigation of sorting mechanisms and by investigating the conditions of sorting a homogeneous mixture in accordance with the specific weight of solid granular particles of its constituents firstly when the mix-

2

ture flows over a sloping surface and secondly it is subjected to a flux of a gas stream rising upwardly through it.

The investigations have shown that sorting by merely flowing the mixture over a sloping surface is practically possible only for mixtures of shallow depth, while the required slope of the surface over which the particles flow depends on the granulometric structure of the mixture.

My investigations have shown furthermore that the optimum sorting obtained through blowing gas through the mixture requires that the speed of the gas through the mixture should be maintained at a constant value within comparatively narrow limits for all the points of the mass subjected to the gas and that its optimum value depends on the density of the constituents of the mixture.

The investigations have also shown that the most efficient results have been obtained through the suitable combination of the above conditions.

According to the present invention there is provided a method of dry sorting mixtures of solid granular particles of different specific weights in accordance with their specific weights, consisting in a first stage causing the mixture to flow under the action of gravity over a porous sloping surface, blowing a gas through said porous sloping surface to fluidize the stream of granular particles causing stream of granular particles to slide during a second stage over a perforated sloping surface through which the sorted particles drop in succession in accordance with the succession of their specific weight.

The stream flowing over the porous surface may have a suitable thickness ranging between 3 and 30 times the average size of the granules and ranges preferably between 3 and 15 times said size.

In order to ensure a uniform speed at all points of the gas stream, the porous surface over which the mixture flows preferably has ports distributed as close to one another as possible, while the size of each port is preferably smaller than that of the finest particles.

The pressure applied to the stream of particles is preferably the lowest required for fluidizing it without any deviation of the upper particles out of the stream.

The slope given to the porous sorting surface is preferably the minimum required to produce a uniform progression of the particles at all points thereof.

The slope given to the lower separating grid also is preferably the minimum required for reliably producing a uniform flow of the stream passing off the porous surface.

Embodiments of my invention will now be described by way of example with reference to the accompanying drawings, in which:

FIGURE 1 is a vertical longitudinal cross-section of the plant according to my invention, showing a sorting channel.

FIGURE 2 is a vertical longitudinal cross-section of the sorting channel provided with a separating grid.

FIGURE 3 is a plan view of the whole arrangement including the sorting channel and separating grid.

FIGURE 4 is a vertical cross-section of a modified embodiment of a sorting channel.

The arrangement in which the mixture is subjected to a sorting treatment includes, as illustrated in FIGURES 1 and 2 a sorting channel 1 of a rectangular cross-section of which the flat bottom 2 is made of finely porous material. Under said bottom, there is provided a pipe 3 through which a gas, for example air, is blown under a uniform pressure throughout the bottom 2.

The channel 1 is set in a manner such that its porous bottom surface may slope by a predetermined angle  $\alpha$  with reference to a horizontal plane. The granular mixture 14 to be sorted is introduced into the channel so as to flow down towards a lower section under the double action

of the slope defined at  $a$  and of the fluidization produced by blowing. For a same mixture, the efficiency of the classification according to specific weights obtained at the lower end of the channels depends on the angle  $a$ , on the value of the pressure of the fluidizing gas taking into account the permeability of the porous surface and length of the channel and the input of solid material entering the channel; said values must be adjusted experimentally with reference to each other in accordance with the above-defined values with a view to obtaining an optimum result. To this end, the channel may be set by any suitable known means at an angle of slope  $a$  which may be adjusted and measured, while the pressure is supplied at adjustable or measurable values depending on the porosity of the bottom and on the dissymmetric composition of the mixture. The input of granular particles is also adjusted to a suitable value through a modification of the thickness of the stream of granular particles. The channel length is defined experimentally beforehand as a function of the nature of the products to be sorted with a view to obtaining a maximum efficiency.

Experience has shown that large differences between the specific weights of the constituents of the mixture to be sorted allow reducing the channel length. If the differences are small said length should be increased.

The channel is of uniform width and is defined as a function of the desired input of solid material by weight taking into account the thickness of the mixture stream and the average specific weight of the mixture to be treated. The width may, if required, be reduced as shown in FIGURE 3 by means of a movable flange 5 of a suitable thickness engaging both sides of the channel.

In order to collect separately at the output end of the channel the constituents which have been classified according to their specific weights during their progression along the channel and which are now arranged in layers of specific weights decreasing from bottom to top within the thickness of the stream of fluidized particles, at the lower end of the channel there is provided a further channel 6 including a separating grid (FIGURES 1, 2, 3). The bottom of said channel 6 is constituted by a slotted or perforated grid 7 wherein the openings are sized so as to match the granulometric composition of the products which are to pass through it. Said channel 6 is set in a manner such that the grid 7 slopes with reference to a horizontal plane by an angle  $b$  which may be adjusted with reference to the angle  $a$  of the slope of the channel 1 in accordance with the nature of the mixture undergoing treatment and the speed of the mixture as it passes out of the sorting channel 1 to ensure a flow at a preferably minimum speed over the separating grid 7.

Under such conditions, there is obtained through the grid 7 in successive portions of the channel 6 a longitudinal classification underneath the channel 6 of the layers of a decreasing weight which were actually distributed vertically within the thickness of the stream of fluidized particles at the output of the channel 1 with an optimum efficiency.

The separation of the different components into as many fractions as may be required in practice may be obtained by arranging underneath the grid flaps 8 which are given a suitable slope, so as to allow the different constituents 15 to be collected to drop into separate containers 9.

The flaps 8 are preferably movable throughout the length of the grid 7, so that it is possible to adjust the grid length corresponding to each constituent in accordance with the requirements of the mixture to be sorted and thereby to adjust the composition of each of said constituents.

It is of advantage to restrict gradually the breadth of the stream of granular particles over the grid as they progress from the input end towards the output end of the grid so as to take into account the gradual decrease of the throughput of granular particles over the grid.

This result may be obtained by way of example in a non-limiting sense as illustrated in FIGURE 3 by two blades 10 perpendicular to the plane of the grid which may be laid over the latter so as to assume the shape of a V the opening of which is adjustable through a flexing or a pivotal movement of said blades about their points of attachment to the sides of the grid at the input end thereof.

Various other modifications of this mixture constituent classifying arrangement may be contemplated all of which draw the classified products out of classified superposed layers of different specific weights extending substantially in horizontal planes.

In certain particular cases depending on the nature of the mixture to be sorted, it is of advantage to accelerate the speed of flow of the upper layer of the stream. Said may be achieved for instance (FIGURE 4) by closing completely or partly by a plate 12 the upper surface of the sorting channel 1.

This results in producing in parallelism with the stream of granular particles a stream of gas tapped off the gas flow blown through the channel bottom and sweeping at a higher speed along the upper surface layer of granular particles. Said speed of flow of the gas and consequently of the granular particles in said surface layer may be adjusted through a vertical shifting of the plate 12 the plane of which may be parallel with that of the porous bottom 2 or may slope with reference to the latter, so as to provide an adjustable cross-section for the flow of the stream of air. It is possible, if required, to increase said speed of flow through a further admission of compressed air under a suitable pressure fed out of a pipe 13 (FIGURE 4), which air is admixed with the air blown through the bottom of the channel 1; it is also possible in contradistinction to reduce the flow of air by closing only a portion of the upper surface of the channel for instance by having a plate 12 which is suitably perforated.

Preferably the porous sloping bottom of the channel 1 comprises an upper layer of the material sold under the registered trademark nylon, said layer being carried by a metal gauze and by a lower sheet of felt.

The slope of the porous channel 1 is adjustable preferably between  $8^\circ$  and  $25^\circ$ . While the slope of the perforated channel 6 is adjustable preferably between  $20^\circ$  and  $40^\circ$ .

For industrial or commercial purposes, preferably a plurality of arrangements may be connected in series each including a sorting channel and separating grid, according to the well-known sorting method for the renewed treatment of intermediate or compound constituents.

I will now give by way of example the results obtained with my improved method.

#### Example 1

The mixture to be treated is a sand of a granulometric composition ranging between 0.15 and 0.35 mm. Its composition as concerns specific weights is as follows:

|                                                          | Percent |
|----------------------------------------------------------|---------|
| (a) Specific weight 2.6 (silica)                         | 43.2    |
| (b) Specific weight about 3.5 (staurotide and/or garnet) | 7.8     |
| (c) Specific weight 4.6 (ilmenite and/or zircon)         | 49      |

The treatment is performed in a sorting channel of a width of 10 cm. and of a length of 90 cm. forming an angle of  $10^\circ 5'$  to the horizontal, under a pressure of blown in air equal to 9 cm. of a water column. The separation is performed over a grid provided with slots of a width of 1.2 mm., sloping at  $31^\circ$  with reference to a horizontal plane. Four fractions are collected after a single passage through the channel with a throughput of 1,080 kg. per hour.

The following tabulae show the distribution of the four fractions F1, F2, F3, F4, being the percentages by weight of the total mixture treated and the composition as to

specific weight for each fraction as compared with the composition of the mixture.

|                                             | Initial mixture | F1  | F2   | F3   | F4  |
|---------------------------------------------|-----------------|-----|------|------|-----|
| Proportions of the fractions by weight----- | 100%            | 17% | 22%  | 38%  | 23% |
| Distribution of the specific weights:       |                 |     |      |      |     |
| a-----                                      | 43.2            | 1.8 | 9.5  | 52.8 | 92  |
| b-----                                      | 7.8             | 6.2 | 12   | 10.4 | 5.2 |
| c-----                                      | 49              | 92  | 79.5 | 27   | 2.8 |

*Example 2*

The preceding fraction F1 is treated again in the same channel with a throughput of 1,120 kg. per hour. After a single passage two fractions are collected F1 and F2, of which the compositions are as follows:

|                                             | Initial mixture | F1   | F2   |
|---------------------------------------------|-----------------|------|------|
| Proportions of the fractions by weight----- | 100%            | 60%  | 40%  |
| Distribution of the specific weights:       |                 |      |      |
| a-----                                      | 1.8             | 0.4  | 3.9  |
| b-----                                      | 6.2             | 3.8  | 9.8  |
| c-----                                      | 92              | 95.8 | 86.3 |

*Example 3*

Concentrated heavy ore consisting of granular particles ranging between 0.15 and 0.40 mm., is treated in the same channel as for the preceding examples, sloping at 8° to the horizontal in a stream of air flowing under a pressure equal to 7 cm. of a water column while the throughput of solid material is equal to 1,160 kg. per hour.

*Initial composition as to specific weights*

|                                                        | Percent |
|--------------------------------------------------------|---------|
| (a) Specific weight 4.5 (ilmenite and/or zircon) ----- | 89      |
| (b) Specific weight 5.1 (monazite) -----               | 11      |

Three fractions F1, F2 and F3 are collected during a single passage in the channel.

The following table discloses the results:

|                                     | Mixture treated | F1  | F2  | F3   |
|-------------------------------------|-----------------|-----|-----|------|
| Distribution by weight-----         | 100%            | 34% | 54% | 12%  |
| Composition as to specific weights: |                 |     |     |      |
| a-----                              | 89              | 77  | 94  | 99.5 |
| b-----                              | 11              | 23  | 5.9 | 0.5  |

Distribution of the product having a specific weight equal to 5----- 100% 74% 29% 0.06%

I claim:

1. A method of dry sorting mixtures of solid granular particles of different specific weights in accordance with their specific weights, comprising the steps of establishing a fluidized bed of mixed granular particles to be sorted above a stationary porous inclined surface with the angle of inclination of the porous surface only enough to cause the fluidized bed to move down along said porous surface by gravity until said particles have vertically stratified into superposed layers whose density decreases from bottom to top, feeding the stratified particles from the lower end of said porous surface to an upper portion of a stationary inclined separating surface having a series of openings therethrough larger than the size of the largest particles to be separated while maintaining the path of the particles unimpeded above said porous and separating surfaces with the angle of inclination of said separating surface greater than that of said porous surface and only enough to cause the particles to move down along said separating surface by gravity, maintaining the pressure below said separating surface no higher than atmospheric, and separately collecting a plurality of fractions of different density below different portions of said separating surface lengthwise along said separating surface.
2. A method as claimed in claim 1, in which said fluidized bed is established by blowing a gas upward through said porous inclined surface under constant pressure.
3. A method as claimed in claim 1, said fluidized bed having a thickness from 3 to 30 times the average size of the granular particles.
4. A method as claimed in claim 1, said fluidized bed having a thickness from 3 to 15 times the average size of the granular particles.

**References Cited**

**UNITED STATES PATENTS**

|           |         |                      |           |
|-----------|---------|----------------------|-----------|
| 1,068,162 | 7/1913  | Payne -----          | 209—466   |
| 2,093,470 | 9/1937  | Morgan -----         | 209—474   |
| 2,303,367 | 12/1942 | Kendall et al. ----- | 209—44    |
| 2,813,630 | 11/1957 | Morrow -----         | 209—474   |
| 2,903,132 | 9/1959  | Berry -----          | 209—475 X |
| 3,007,577 | 11/1961 | Putman -----         | 209—474 X |

HARRY B. THORNTON, Primary Examiner.

TIM R. MILES, Assistant Examiner.